

## UNITED STATES PATENT OFFICE

2,559,305

## MANUFACTURE OF TANNING SUBSTANCES

Michael Mangold, Frankenau, near Aspang, Austria, and Fritz Neuber, deceased, late of Vienna, Austria, by Hilda Neuber, administratrix, Vienna, Austria

No Drawing. Application February 20, 1948, Serial No. 9,953. In Germany May 2, 1944

Section 1, Public Law 690, August 8, 1946  
Patent expires May 2, 1964

6 Claims. (Cl. 260—124)

1

This invention relates to a process for producing tanning substances.

Hitherto it was known to use sulphite waste lye as an additional tanning substance for so-called pseudo-tannings. Another utilization of such lyes, likewise merely as an additional tanning substance, consists in liberating the lyes from lime salts and iron by an acid treatment and to convert them into a commercial product by extracting them and concentrating the extract. Moreover, a genuine tanning substance is known made from dry, dust-like waste lye by condensation with formaldehyde, sulphonation and neutralization; this substance is used as tanning agent without further additions. In all processes, the tanning effect of the ligno-sulphonic acids is used to a slight extent only and a recovery of the sulphur combined with the lignin was not provided.

The main object of this invention is to provide a process for producing tanning substances from sulphite cellulose waste lye or the residue thereof, wherein the tanning effect of the ligno-sulphonic acids is utilized practically in a complete manner.

A further object of this invention is to provide a process for producing tanning substances of the class referred to above, wherein the sulphur combined with the lignin is recovered.

Another object of this invention is to provide a process for producing tanning substances of the class referred to above, wherein the tanning substances obtained represent a means or agent which can be used by themselves, that is without any other additional chemical agents, for tanning purposes.

A further object of this invention is to provide a process for producing tanning substances of the class referred to above, wherein besides these tanning substances, other valuable substances, such as hydroxy- and alkoxy-aldehydes, especially vanillin, sugar acting as a reducing agent and organic acids, are obtained as by-products. Other objects and advantages of this invention will be apparent from the following description.

We have found that when a sulphite-cellulose waste lye or its residue is carefully treated with alkali at a temperature below 100°C., the sulphonic groups are disengaged for the greatest part from the salts of the ligno-sulphonic acids while phenolic OH-groups are introduced, with a concurrent enlargement of molecules owing to a simultaneous condensation. The tanning substances obtained by this careful treatment from

2

the reaction product by double decomposition of the alkali salts with acids, are soluble in water. The process according to this invention, is therefore particularly advantageous in that it directly yields tanning substances in a very simple manner, said substances being easily soluble in water and in strong acids. Such substances can be employed for tanning purposes according to usual methods without any after-treatment.

10 The tanning substances are obtained by decomposition of the alkali salts with acids, from the reaction product which accumulates owing to the effect of alkali, as a dark-brown, thick liquid, at the said temperatures. Since sodium chloride salts out the tanning substances, the reaction product is preferably treated with hydrochloric acid, whereby the alkali salts of the compounds of the tanning substances are decomposed and the liberated tanning substances are precipitated by the sodium chloride formed. These tanning substances are insoluble in the cold, but easily and practically completely soluble in the heat and after having been dissolved in the heat, they remain in a dissolved state, even when cooled down. Since in this careful treatment, the sulphonic groups are disengaged for the greatest part from the salts of the ligno-sulphonic acids and a mixture with the alkali salts of the compound of tanning substances is formed, 20 all sulphur compounds of organic character are contained in a very reactive form in this mixture. By the action of acid, they are destroyed almost completely and gaseous sulphur dioxide is obtained. The latter may be directly supplied to a cellulose manufacturing plant.

For example, the residue of sulphite waste lye, thickened to 30% Baumé, is heated to a temperature of 60° to 80°C. and, while stirring, mixed with 40 parts of waste lye by volume (per 100 parts) of solid NaOH or with an equivalent amount of caustic soda solution and then well stirred in the heat with admission of air for several hours. Then, while stirring continues, the solution is neutralized by adding hydrochloric acid drop by drop; the escaping SO<sub>2</sub> is collected and the tanning substance agglomerates; when heated for a longer time, it precipitates in form of small grains which may be filtered off in the cold, and are washed, dried and pulverized. About 60 to 70 per cent of tanning substance, calculated on the organic dry substance of the initial material, are thus obtained. Similar results are obtained by heating 130 parts of spruce-wood sulphite waste lye of 34.2 Baumé with 67 30 parts of strong 60 per cent lye, or 128 parts of

beech-wood sulphite waste lye of 33° Baumé with 40 parts of solid caustic soda at 90 to 100° C., while stirring, for 6 to 8 hours.

The obtained tanning substance can be used by itself, without addition of other substances, for tanning purposes and is practically completely soluble in warm water with a yellow-brown color. The solution has a pH-value of 3 to 4 and may be used according to the usual tanning prescriptions. The tanning substance is absorbed almost completely by the normally treated hides. The leather obtained is light-brown, has a slightly aromatic smell, good strength, and soft quality.

A further advantage of our process consists in that owing to the careful low temperature treatment with alkali, not only the tanning substances of advantageous properties, but other valuable products can be obtained in the course of this process. These products are destroyed completely or for the greatest part, if tanning substances are obtained from sulphite waste lye by a more intensive action of alkali. Such by-products are, first of all, hydroxy- and alkoxy-aldehydes, especially vanillin, as well as sugar acting as a reducing agent, and organic acids. Hydroxy- and alkoxy-aldehydes are obtained from the mother liquor remaining after the separation of the tanning substance, according to methods known per se, e. g. by extraction with organic solvents or by steam distillation, a remaining solution rich in reducing, sugar-like substances and organic acids being obtained.

In order to avoid losses of hydroxy- and alkoxy-aldehydes when separating tanning substances from the mixture obtained by an alkali treatment of the sulphite waste lye or the like at relatively low temperatures, acid, preferably hydrochloric acid, is added in such an amount that only bisulphite and a small quantity of free sulphur dioxide are formed in the acidified mixture, whereas the presence of free mineral acid is avoided, since such acid would decompose the bisulphite compounds of the hydroxy- and alkoxy-aldehydes split off from the lignin in the secondary reaction, and would result in a separation of the aldehydes together with the tanning substance in insoluble form. The acidification of the mixture for separating the tanning substance is therefore only carried to a pH-value of 5. Only after the separation of the tanning substance has occurred, the solution should be further acidified. If, for instance, an extraction process is used to obtain the aldehydes, the mother liquor deprived from the tanning substance, is adjusted to a pH-value lower than 5, preferably to a pH-value between 2 and 3. Before, or after, the aldehydes are obtained, the solution may be evaporated and the mineral salts, normally sodium chloride, may be obtained by crystallizing and centrifuging or the like. The separated salts may be used as tanning salts.

The residue which may be concentrated by evaporation at a suitable pH-value such as a pH-value of 5, represents a rather thick liquid of greyish-brown color, which still contains large amounts of highly reducing, sugar-like substances, as well as various organic acids and may be employed as a reducing agent for technical purposes, for instance to reduce metallic salts in galvanic processes, manufacture of dyes, vat-dyeing and so on, and can substitute the substances, such as glucose, hyposulphite and the like, used heretofore in these domains.

The process according to the invention has therefore the advantage of a practically complete utilization of the sulphite cellulose waste lye, since the following substances are obtained:

(a) A practically completely soluble tanning substance representing 60 to 70 per cent. of the organic dry substance of the sulphite cellulose waste lye or its residue, which substance may, under normal tanning conditions, be employed as the only tanning means in the process.

(b) A large part of the sulphur contained in the initial material, particularly of the organically combined sulphur, in the form of sulphur dioxide.

(c) A mixture of hydroxy- and alkoxy-aldehydes, which may be further decomposed according to known methods.

(d) Solid alkali metal salts formed from the reagents used in the process, which salts may be used as tanning salts.

(e) A liquid reducing agent of high effect.

#### Examples

(1) 125 parts by weight of a thickened sulphite spirit residue containing 32.4 per cent. organic dry substance, are treated at normal temperature in a kneader with 40 parts of solid caustic soda which are gradually added. By proper control of the alkali addition, a temperature of 90 to 100° C. is reached which is maintained throughout the following 6 to 8 hours. During that period, the mixture is being stirred and becomes thicker and darker. It is then diluted with water in the amount of one third of the volume, whereafter a pH-value of 5 is adjusted with hydrochloric acid, the disengaged tanning substances are filtered off and washed in the cold with 0.5 per cent. hydrochloric acid and thereafter with water. 28 parts by weight of a dry tanning substance are obtained. The mother liquor remaining from the filtration is mixed with the washing liquid and heated, while the escaping sulphur dioxide is collected. From the remaining acid solution, in which the pH-value is adjusted to 2-3, the hydroxy- and alkoxy-aldehydes liberated from their bisulphite compounds are obtained as yellow oils by known extraction methods with organic solvents (chloroform, ether, methylene chloride and so on). The yield amounts to 3 parts by weight. The aqueous solution is then neutralized with alkali and concentrated by evaporation to such an extent that the dissolved sodium chloride is precipitated. There remain 18 parts by weight of a liquid which may be used as a reducing agent.

(2) 130 parts by weight of a thickened spruce-wood sulphite waste lye containing 34.7 per cent. organic dry substance are stirred at the conditions of the Example 1 with 67 parts by weight of 60 per cent. strong lye at 90 to 100° C. for 6 to 8 hours, and the resulting mixture is worked up according to Example 1. The yields amount to 30 parts by weight of tanning substance, 5 parts by weight of a mixture of aldehydes, 20 parts by weight of a reducing agent.

(3) 128 parts of a thickened beech-wood sulphite waste lye containing 38 per cent. of organic dry substance are stirred at the conditions of Example 1 with 40 parts of solid caustic soda at 90 to 100° C. for 6 to 8 hours. By further working up the resulting mixture according to Example 1, 31 parts by weight of a tanning substance, 8 parts by weight of a mixture of aldehydes.

hydes, and 18 parts by weight of a reducing agent are obtained.

In order to separate the tanning substances from the solution diluted with water, relatively large amounts of mineral acids are consumed in this process, irrespective of the particular conditions maintained in the alkali treatment, since the entire amount of alkali subjected to the reaction must be combined with the acid, before the tanning substance is liberated from its alkali compounds. However, it is possible to separate the tanning substances from the solution under conditions that will enable us to save a considerable amount of mineral acid, with concurrent, partial recovery of the excessive alkali in form of valuable compounds.

For this purpose the diluted solution resulting from the treatment of the sulphite waste lye or its residue with alkali is subjected to a saturation with carbon dioxide or gases containing carbon dioxide, before the tanning substances are liberated by the acid treatment. The process is preferably carried out so that the saturation with carbon dioxide is effected in two stages by introducing first carbon dioxide, until a pH-value of 9 is attained; in this stage substantially sodium sulphite and sodium sulphate are precipitated together with slight amounts of soda. After separating the mixture of salts (fraction I) the saturation with carbon dioxide is continued in a second stage, until a pH-value of about 7.5 is reached. A mixture of bicarbonates with some soda precipitate is thus obtained, which includes at the same time a considerable amount of saponine substances of high lathering power, (fraction II).

By the described saturation with carbon dioxide and the preliminary separation of the precipitated salts, about two thirds of the alkali present are removed from the solution so that the amount of mineral acid necessary for complete combination with the remaining alkali will be only one third of the amount required otherwise. After elimination of the salts formed in the reaction, the solution still contains the alkali compounds of the tanning substances, and, especially when working up beech-wood, considerable amounts of sodium acetate. For liberating the tanning substances, the solution is now acidified, preferably up to a pH-value of 3.5 in a manner known per se. The acidification may be effected by mineral acids, such as hydrochloric, sulphuric or phosphoric acid. The use of sulphuric or phosphoric acid to liberate the tanning substances from their alkali compounds is particularly advantageous, since in such a case the liquid which is obtained, after the precipitated substances are filtered or centrifuged off, may be subjected to a distillation, if desired after being strongly acidified once more, in order to obtain acetic acid in the distillate.

The carbon dioxide required in the course of the process for saturation and preliminary separation, is available in large quantities in paper mills and cellulose factories. There, the sulphite waste lye to be worked up accumulates, since in the manufacture of the waste lye of calcium bisulphite from lime stone and sulphurous acid, this lye being used for disintegrating purposes, carbon dioxide escapes from the lye-towers as a waste gas. The mixture of sodium sulphite and sodium sulphate, accumulating as fraction I can be returned into the process by admixing this mixture of salts to the water in the lye-towers. The mixture accumulating as fraction

II in the preliminary separation may be used as a washing means or as an additional washing means due to its content of carbonates, bicarbonates and saponine-like substances.

5. In the claims, the expression "concentrated caustic alkali," when not otherwise specified, is intended to define concentrations in the order of about 30 parts by weight of caustic alkali (corresponding to about 40 parts by volume, as given in the examples) per 100 parts of sulphite cellulose waste lye of about 30° Bé.

6. The expression "sulphite cellulose waste lye" in the claims is intended to define a concentrated waste lye of about 30° Baumé including waste lye residues which remain after the extraction of spirit or the like.

What we claim is:

1. A process for producing tanning substances from sulphite cellulose waste lye, which comprises treating said waste lye in form of a concentrated liquor of about 30° Bé. with concentrated caustic alkali solution containing at least 60 per cent of alkali hydroxide, maintaining the alkaline solution under atmospheric pressure at 25 a temperature ranging from 60 to 100° C. for several hours, precipitating from the alkaline solution the tanning substances which formed during said treatment by addition of hydrochloric acid in an amount imparting a pH-value of about 5 to the resulting liquid, and removing the tanning substances from said liquid.

2. A process for producing tanning substances from sulphite cellulose waste lye, which comprises treating said waste lye in form of a concentrated liquor of about 30° Bé. with caustic alkali in a ratio of about 30-32 parts of caustic alkali, calculated as solid alkali hydroxide, per 35 100 parts of said concentrated liquor, said liquor containing from about 30-38 per cent of dry organic substances, maintaining the alkaline solution thus formed under atmospheric pressure at a temperature ranging from 60 to 100° C. for several hours, precipitating from the alkaline solution the tanning substances formed during the treatment by addition of hydrochloric acid in an amount imparting a pH-value of about 5 to the resulting liquid, and removing the tanning substances from said liquid.

3. A process for producing tanning substances from sulphite cellulose waste lye, which comprises treating said waste lye in form of a concentrated liquor of about 30° Bé. with concentrated caustic alkali at a temperature ranging from 60 to 100° C. for several hours under atmospheric pressure, precipitating from the alkaline solution the tanning substances formed during the treatment by addition of hydrochloric acid in an amount imparting to the resulting liquid a pH-value of about 5, removing the tanning substances from said liquid, adding more acid to bring the pH-value of the liquid to 2-3, and extracting therefrom the hydroxy- and alkoxy-aldehydes present therein.

4. A process for producing tanning substances from sulphite cellulose waste lye, which comprises treating said waste lye in form of a concentrated liquor of at least 30° Bé. with concentrated caustic soda at a temperature ranging from 60° C. to 100° C. for several hours, saturating the alkaline solution with carbon dioxide in two stages, introducing the carbon dioxide in a first stage until a pH-value of about 9 is reached in the solution, separating from the liquid the formed mixture of sodium sulphite, sodium sulphate, and sodium carbonate, then

introducing carbon dioxide in said second stage until the pH-value reaches about 7.5, separating from the liquid the formed carbonates, bicarbonates, and saponine-like substances, thereafter acidifying the liquid for precipitation of the tanning substances and separating the same from the liquid.

5. A process according to claim 4, wherein the caustic soda is added in form of solid NaOH in a ratio of about 30-32 parts to 100 parts of the concentrated liquor.

6. A process according to claim 4, wherein the caustic soda is added in form of a concentrated solution of at least 60 per cent NaOH, in an amount of about 30-32 parts of NaOH for 100 parts of concentrated liquor.

MICHAEL MANGOLD.

HILDA NEUBER,

*Administratrix of the Estate of Fritz Neuber,  
Deceased.*

### REFERENCES CITED

The following references are of record in the file of this patent:

#### UNITED STATES PATENTS

| Number       | Name         | Date          |
|--------------|--------------|---------------|
| 263,797      | Mitscherlich | Sept. 5, 1882 |
| 940,394      | Kumpfmiller  | Nov. 16, 1909 |
| 1,147,245    | Hurt         | July 20, 1915 |
| 10 1,303,176 | Drewson      | May 6, 1919   |
| 1,571,873    | Blackadder   | Feb. 2, 1926  |
| 1,592,062    | Baker        | July 13, 1926 |
| 1,629,448    | Drewson      | May 17, 1927  |
| 2,241,306    | Honig        | May 6, 1941   |